

## UNITED STATES PATENT OFFICE

2,027,807

## COPPER BASE ALLOY

Henry L. Burghoff, Yalesville, and David E. Law-  
son, Waterbury, Conn., assignors to The Chase  
Companies, Incorporated, Waterbury, Conn., a  
corporation

No Drawing. Application May 13, 1932,  
Serial No. 611,238

## 11 Claims. (Cl. 75—1)

This invention relates to improvement in copper-base alloys, that is to say, alloys in which copper is the major constituent, and has for its main object the improvement of the physical properties of such alloys, as will hereinafter appear.

We have discovered that by including relatively small quantities of tellurium in copper-base alloys, such as ordinary brasses, aluminum brasses, 10 tin bronzes, etc., the tellurium serves to inhibit grain growth and thus serves to provide in the metal a grain structure materially smaller than would ordinarily be the case, were the tellurium absent. Our investigations have shown that the 15 tellurium has no appreciable effect on the temperature of incipient recrystallization, or, in other words, the tellurium does not raise the temperature of initial softening. The tellurium has, however, a very marked effect on the rate of 20 grain growth after recrystallization, inasmuch as it acts, as above pointed out, as an inhibitor, tending to prevent grain growth, which ordinarily accompanies high temperature annealing. It will thus be seen that the tellurium imparts to the 25 metal highly desirable characteristics of softness and ductility without, however, producing an unduly-coarse crystal or grain structure which would be objectionable for many finishing operations. With the smaller grain size, due to the 30 presence of tellurium, lower finishing costs result.

We have also discovered that by including tellurium in copper-base alloys, the modulus of elasticity of the same may be lessened to a degree sufficient to render the material more flexible 35 than would otherwise be the case where such a quality is desired.

Furthermore, we have discovered that by combining tellurium with certain copper-base alloys, the machinability of such alloys is distinctly improved. This improved machinability of tellurium-bearing copper alloys is evidenced in several ways, such, for instance, as during a sawing operation at 40 which time it will be found that such alloys cut easily and rapidly with substantially no tendency to seize or bind. When being drilled, these alloys cut rapidly and cleanly and the cut chips do not clog the drill. By way of illustration, it may be 45 stated that it was found that an average of seventy cuts of a power-saw were required to sever a rod composed of 90% copper and 10% zinc, while only thirty-five saw-cuts were required to sever a similar rod composed of 89.8% copper, 10% zinc and 0.2% tellurium. A rod composed of 89% copper, 10% zinc and 1% aluminum, required seventy-nine saw-cuts to be sev-

ered, while a substantially-similar rod containing 0.2% tellurium required only forty-six saw-cuts for the same operation.

Practically all types of machining operations may be performed upon our improved alloy without occasioning appreciable chattering or vibration, though as might be expected, the alloy becomes heated when being machined. However, this heating of our improved alloy is to a much less extent than would be the case with copper-base alloys having no appreciable tellurium content. It is common knowledge that ordinary copper-base alloys are heated to such degree by any extensive machining operation that handling the same with bare hands is inconvenient or impossible, but we have found that similar alloys containing tellurium in proper proportions are heated by machining to such a relatively-slight degree that they may be freely handled during such operations.

Our improved alloy is characterized by a preponderance of copper and from 0.08% to 1.75% inclusive of tellurium, together, if desired, with other elements such, for instance, as zinc, tin, aluminum, nickel, cadmium, manganese, silicon, 25 cobalt, etc.

Preferably, our improved alloy should contain between 0.20% and 0.50% tellurium, as we have found that within that range the alloy possesses most of the desirable physical properties without undue brittleness, though as before pointed out, we have found that a copper-base alloy containing from 0.08% to 1.75% tellurium possesses marked advantages over similar alloys containing tellurium in amounts outside the last-mentioned 35 range.

The following table sets forth alloys which are illustrative of some of the various combinations of materials in accordance with our invention:

|             | A     | B     | C     | D     | E     | F     | G     |    |
|-------------|-------|-------|-------|-------|-------|-------|-------|----|
| Copper %    | 56.00 | 95.00 | 80.00 | 92.00 | 98.80 | 98.80 | 90.00 | 45 |
| Tellurium % | 0.30  | 0.20  | 0.50  | 0.50  | 0.10  | 0.10  | 0.50  |    |
| Zinc %      | 43.00 |       |       |       |       |       |       |    |
| Tin %       |       | 4.73  |       |       |       |       |       |    |
| Aluminum %  |       |       | 19.40 | 7.42  |       |       |       |    |
| Nickel %    |       |       |       |       | 1.00  |       |       |    |
| Cadmium %   |       |       |       |       |       |       | 0.40  |    |
| Manganese % |       |       |       |       |       | 3.00  |       |    |
| Silicon %   |       |       |       |       | 0.10  | 0.10  | 0.10  | 50 |
| Misc. %     | 0.10  | 0.07  | 0.10  | 0.08  |       |       |       |    |

Microscopic examination has shown that in most of the alloys above mentioned, the tellurium is present, largely at least, in a second phase from 55

the usual alpha phase of high-copper alloys. This second phase probably contains some form of copper-telluride.

In making up our improved alloy, any of the well-known methods of combining the constituent parts may be employed such, for instance, as by directly adding the tellurium or by first alloying the tellurium with one or more of the components of the material in question to produce a high tellurium-content alloy for later dilution.

Although reference is made herein to certain specific alloys, it is to be understood that our invention is not limited to the proportions recited, but only to the proportions set forth in the appended claims.

We claim:

1. A ductile copper-base alloy comprising copper and tellurium, with the copper content being at least 75% and the tellurium being present in an amount from 0.08% to 1.75% inclusive, the said alloy being characterized by substantially improved machinability over what the alloy would possess in the absence of said tellurium.

2. A ductile copper-base alloy comprising copper and tellurium, with the copper content constituting 90% or more of the combined copper and tellurium, and the tellurium being present in an amount from 0.08% to 1.75% inclusive, the said alloy being characterized by substantially improved machinability over what the alloy would possess in the absence of said tellurium.

3. A ductile copper-base alloy comprising copper and tellurium, with the copper content constituting 90% or more of the combined copper and tellurium, and the tellurium being present in an amount from 0.20% to 0.50% inclusive, the said alloy being characterized by substantially improved machinability over what the alloy would possess in the absence of said tellurium.

4. A ductile copper-base alloy comprising copper, a minor amount of zinc and tellurium, the copper content being more than 50% and the tellurium being present in an amount from 0.08% to 1.75% inclusive, the said alloy being characterized by substantially improved machinability over what the alloy would possess in the absence of said tellurium.

5. A ductile copper-base alloy comprising copper, a minor amount of zinc and tellurium, the

copper content being more than 50% and the tellurium being present in an amount from 0.20% to 0.50% inclusive, the said alloy being characterized by substantially improved machinability over what the alloy would possess in the absence of said tellurium.

6. A ductile copper-base alloy comprising copper, a minor amount of tin and tellurium, with the copper content being more than 50% and the tellurium being present in an amount from 0.08% to 1.75% inclusive, the said alloy being characterized by substantially improved machinability over what the alloy would possess in the absence of said tellurium.

7. A ductile copper-base alloy comprising copper, a minor amount of tin and tellurium, with the copper content constituting 90% or more of the combined copper and tellurium, and with the tellurium being present in an amount from 0.20% to 0.50% inclusive, the said alloy being characterized by substantially improved machinability over what the alloy would possess in the absence of said tellurium.

8. Copper or copper base alloys containing from approximately .1% to 1.75% of tellurium and being characterized by substantially improved machinability over that which would exist in the absence of said tellurium.

9. An alloy of copper and silicon containing from approximately .08% to 1.75% of tellurium and having a silicon content of approximately 3% and the balance substantially copper, the said alloy being characterized by substantially improved machinability over what the alloy would possess in the absence of said tellurium.

10. A copper-base alloy containing more than 75% copper, silicon, and approximately 0.08% to 1.75% tellurium, the said alloy being characterized by substantially improved machinability over what the alloy would possess in the absence of said tellurium.

11. A copper-base alloy containing more than 90% copper, approximately 3% silicon, and approximately 0.08% to 1.75% tellurium, the said alloy being characterized by substantially improved machinability over what the alloy would possess in the absence of said tellurium.

HENRY L. BURGHOFF.  
DAVID E. LAWSON. 50